

## UNITED STATES PATENT OFFICE

2,346,090

## PHOTOGRAPHIC BLEACH-OUT LAYER

Henry C. Staeble, Rochester, N. Y., assignor to  
 Eastman Kodak Company, Rochester, N. Y., a  
 corporation of New Jersey

No Drawing. Application August 19, 1942,  
 Serial No. 455,343

5 Claims. (CL. 95—6)

My invention relates to light-sensitive layers for photography, and more particularly to light-sensitive layers for the so-called "bleaching out" process of photography.

As is well known, the bleaching-out process of photography primarily consists of exposing to light a layer containing a dye capable of being decolorized under influence of light. Various substances have been used in this process for the purpose of speeding up the printing of the photographic layer and the bleaching of the dye therefrom. For instance, hydrogen peroxide has been used to accelerate the bleaching, but due to the fact that it rapidly decomposes into oxygen and water, it is of little or no use. Similarly, metal peroxides such as barium peroxide have been tested as bleaching accelerators, but have been found to be of little or no use.

In a bleaching-out process in which the accelerator is incorporated in the photographic layer along with the dye, the special characteristics which the bleaching accelerator must have are that it will keep indefinitely in intimate contact with the dye without adverse effects upon the dye, and yet is or may be caused to be available when required for bleaching. To meet these requirements, the accelerator should be relatively stable and non-volatile. Moreover, after the accelerator has served its purpose, it should be readily removable from the layer to prevent further bleaching of the dye in the unexposed area of the layer. It is now apparent why a relatively unstable peroxide such as hydrogen peroxide is unsuitable for the purpose. Peroxide compounds relatively more stable than hydrogen peroxide, such as solid peroxides, would be suitable for use in the process since they have relatively low vapor pressures and are, therefore, substantially non-volatile under ordinary conditions.

One object of the present invention is to provide a photographic material for use in the bleaching-out process of photography.

Another object is to provide bleaching accelerator compounds of particular use in bleaching-out layers.

I have discovered a class of peroxide compounds, namely, solid organic peroxides which are eminently suitable for use in the bleaching-out process and especially suitable for incorporation into bleaching-out layers. Typical solid organic peroxides which are found to be suitable for use in my invention are, for example, benzoyl peroxide, acetyl benzoyl peroxide, ascaridol,

acetyl peroxide, and tetratin peroxide *Helv. Chim. Acta* 15, 1390 (1932), and others.

These peroxides, especially benzoyl peroxide, have the property of being relatively stable in the dry state; however, upon treatment with moisture they gradually decompose into organic acid and hydrogen peroxide. This property is especially useful in my process as will be apparent from the following description.

In the manner of my invention the peroxide compound is incorporated into the photographic layer along with the dye and the layer kept in the dry state until it is desired to make an exposure, then the layer is first moistened, then exposed, and finally treated with further moisture in the absence of strong light to decompose the residual peroxide compound.

The photographic layer may contain as the binding agent a high molecular weight colloidal material such as natural or synthetic resins, cellulose esters and the like. For example, cellulose nitrate or acetate, cellulose mixed esters, such as cellulose acetate propionate, resins such as polyvinyl acetate, cellulose ethers, etc. are suitable.

The following examples illustrate my invention.

## Example 1

30 A baryta paper is coated with a solution of the following composition:

|                     | Grams |
|---------------------|-------|
| Cellulose nitrate   | 4.0   |
| Amyl acetate        | 75.57 |
| 35 Methyl alcohol   | 9.5   |
| Acetone             | 9.5   |
| Triphenyl phosphate | 0.6   |
| Methylene Blue      | 0.03  |
| Benzoyl peroxide    | 0.8   |

40 After curing the paper it is stored in a dry place until required for use. The cellulose nitrate used in the above formula is a low viscosity highly alcohol soluble nitrate of nitrogen content of about 11 per cent. Before exposure the paper is moistened by exposure to humid air and following this exposed to strong light under a suitable pattern and finally exposed further to moist air to decompose the peroxide compound remaining in the layer. The paper is then dried. Where the colored layer has been exposed to light, the dye will be markedly destroyed. The unexposed portions will be relatively unaffected. The principal function of the peroxide is to increase the rate of bleaching, that is, by having

the peroxide present, the dye is bleached in a fraction of the time required when no peroxide is used.

*Example 2*

A baryta paper is coated with a subbing layer of cellulose nitrate from a subbing composition as shown in Example 1, except containing no dye or peroxide. Over the nitrate subbing layer is coated a solution of the following composition:

|                   | Grams |
|-------------------|-------|
| Polyvinyl acetate | 5.0   |
| Methyl alcohol    | 94.17 |
| Methylene Blue    | 0.03  |
| Benzoyl peroxide  | 0.8   |

If desired, the paper may first be coated with the composition of Example 1, minus either the dye or peroxide compound, followed by a coating from the solution of Example 2 containing either dye or peroxide compound depending upon which was used in the undercoat. After curing, the paper is stored in a dry place. The bleaching-out paper thus prepared may be processed as described in Example 1.

*Example 3*

A baryta paper is coated with a subbing layer from a composition such as shown in Example 1, preferably containing no dye or peroxide compound. This subbing layer is then overcoated with a bleaching-out layer containing cellulose acetate 38 per cent acetyl, as the binding agent, from the following solution.

|                   | Grams |
|-------------------|-------|
| Cellulose acetate | 3     |
| Acetone           | 69.17 |
| Methyl alcohol    | 27    |
| Benzoyl peroxide  | 0.8   |
| Methylene Blue    | 0.03  |

In the production of other bleaching-out papers prepared in a manner similar to that shown in the preceding examples, other organic peroxide compounds may be used in place of benzoyl peroxide, and similarly, other dyes may be substituted for the particular dye of the examples. In addition, if it is so desired, instead of coating a baryta paper one may use for the support a cellulose ester as, for example, cellulose nitrate and coat this support with a solution of dye, organic peroxide compound and cellulosic or resin binder from a solvent combination such as shown in Example 1. It is not necessary that the coating composition be entirely free from water since peroxides are slowly decomposed in water. Ac-

ordingly, other binding agents which can be coated from aqueous organic solvent solution are suitable for use in the layers of my invention.

Other dyes suitable for use in the bleaching-out layers of my invention may for example be Rhodamine, Curcumin, Brilliant Green, Pyronine G, Rosinduline, etc.

Obviously, my invention is not limited to the foregoing examples or the described methods given therein, and it is to be understood that the disclosure herein is by way of example and that I consider as included in my invention all modifications and equivalents falling within the scope of the appended claims.

What I claim is:

1. The method of forming a photographic layer for the bleaching-out process which comprises dissolving in organic solvent medium a binding agent, a bleaching-out dye, and a solid organic peroxide compound as an accelerator for bleaching said dye, and coating a layer from the composition.

2. The method of forming a photographic layer for the bleaching-out process which comprises dissolving in organic solvent medium substantially free of water, a binding agent, a bleaching-out dye, and a solid organic peroxide compound as an accelerator for bleaching said dye, and coating a layer from the composition.

3. The method of forming a photographic layer for the bleaching-out process which comprises dissolving in organic solvent medium a binding agent, a bleaching-out dye, and benzoyl peroxide as an accelerator for bleaching said dye, and coating a layer from the composition.

4. The method of forming pictures in the bleaching-out process of photography which comprises moistening a photographic layer having a binding agent and uniformly dispersed therein a bleaching-out dye and a solid organic peroxide as an accelerator for bleaching said dye, exposing said layer through a pattern, and treating said layer with additional moisture to decompose any undecomposed peroxide in the layer.

5. The method of forming pictures in the bleaching-out process of photography which comprises moistening a photographic layer having a binding agent and uniformly dispersed therein a bleaching-out dye and benzoyl peroxide as an accelerator for bleaching said dye, exposing said layer through a pattern, and treating said layer with additional moisture to decompose any undecomposed peroxide in the layer.